

## UNITED STATES PATENT OFFICE

2,014,487

AZODYESTUFFS INSOLUBLE IN WATER AND  
FIBERS DYED THEREWITH

Werner Zerweck and Karl Schütz, Frankfort-on-the-Main-Fechenheim, Germany, assignors to General Aniline Works, Inc., New York, N. Y., a corporation of Delaware

No Drawing. Application May 15, 1934, Serial No. 725,820. In Germany May 23, 1933

8 Claims. (Cl. 260—95)

The present invention relates to new azodyestuffs insoluble in water more particularly to such corresponding to the general formula



(wherein  $\text{R}_1$  means an aryl or aralkyl radical and  $\text{R}_2$  a combining component of the group consisting of arylamides of acyl-acetic acids and ortho-hydroxy-aryl-carboxylic acids).

The dyestuffs may be prepared by combining in substance or on the fiber or on a substratum a diazocompound of an amine



with a combining component  $\text{R}_2$  ( $\text{R}_1$  and  $\text{R}_2$  have the aforesaid significance). The dyeings obtained with these dyestuffs are distinguished by bright shades and a good fastness.

In order to further illustrate our invention the following examples and table are given; but we wish it however to be understood that our invention is not limited to the particular products nor reacting conditions mentioned therein.

## Example 1

50 grams of cotton yarn are treated for half an hour with 1 liter of the following impregnating bath (a), squeezed or centrifugated; the wet material is then dyed in the developing bath (b). Thereupon it is rinsed, soaped at the boil and dried.

## (a) Impregnating bath:

7 grams of (2'-hydroxy-3'-naphthoylamino)-benzene are dissolved at boiling temperature with

10 cc. of Turkey red oil of 50% strength and 10.5 cc. of caustic soda solution of 34° Bé. To the solution

2.7 cc. of formaldehyde of 30% strength are added and the whole is then made up with cold water to

1 liter.

## (b) Developing bath:

1.4 grams of 4'-chlorophenyl-2-amino-benzyl-sulfone are diazotized with 15 cc. of hydrochloric acid normal and 5 cc. of a normal sodium nitrate solution. After the addition of 20 cc. of glacial acetic acid the hydrochloric acid is neutralized by means of a solution of sodium acetate. Then 30 grams of sodium chloride are added and the whole is made up with water to

1 liter.

A vivid golden-orange dyeing of remarkable fastness qualities is obtained.

## Example 2

Into an aqueous suspension of 26.3 grams of 2'-hydroxy-3'-naphthoyl-amino-benzene, prepared by dissolving the said arylide in an alcoholic caustic soda solution, diluting with water and neutralizing with acetic acid, a diazo solution, prepared in the usual manner from 26.1 grams of 4'-tolyl-2-amino-benzyl-sulfone, is allowed to run in. The bright scarlet-red dyestuff separates in the form of flakes. When coupling is finished it is filtered with suction and washed until neutral.

In the same manner similar clear yellowish orange shades may be obtained according to one of the usual printing methods.

The following table shows the shades of some further dyestuffs obtained according to the present process:

| Diazo-component:                               | Coupling component:                                                                                         | Shade:                                                |
|------------------------------------------------|-------------------------------------------------------------------------------------------------------------|-------------------------------------------------------|
| 4'-chlorophenyl-2-amino-benzyl-sulfone.<br>Do. | 1-(2'-hydroxy-3'-naphthoyl-amino)-2-methoxy-benzene.<br>1-(2'-hydroxy-3'-naphthoyl-amino)-4-chloro-benzene. | Scarlet.<br>Full yellowish orange.<br>Bright scarlet. |
| Do.                                            | 1-(2'-hydroxy-3'-naphthoyl-amino)-2-methyl-4-chloro-benzene.                                                | Bright scarlet.                                       |
| Do.                                            | 1-(2'-hydroxy-3'-naphthoyl-amino)-3-nitrobenzene.                                                           | Bluish red.                                           |
| Do.                                            | 2-(2'-hydroxy-3'-naphthoyl-amino)-naphthalene.                                                              | Orange.                                               |
| Do.                                            | 4, 4'-di-(acetoacetyl-amino)-3', 3'-dimethyl-diphenyl.                                                      | Vivid greenish yellow.                                |
| 4'-chlorophenyl-4-amino-benzylsulfone.<br>Do.  | (2'-hydroxy-3'-naphthoyl-amino)-benzene.                                                                    | Red.                                                  |
| Do.                                            | 1-(2'-hydroxy-3'-naphthoyl-amino)-2-methoxy-benzene.                                                        | Yellowish red.                                        |
| 4'-methylphenyl-2-amino-benzylsulfone.<br>Do.  | 1-(2'-hydroxy-3'-naphthoyl-amino)-4-chloro-benzene.                                                         | Red.                                                  |
| Do.                                            | 1-(2'-hydroxy-3'-naphthoyl-amino)-4-methylbenzene.                                                          | Vivid scarlet.                                        |
| Do.                                            | 2-(2'-hydroxy-3'-naphthoyl-amino)-naphthalene.                                                              | Do.                                                   |
| 55                                             | 1-(2'-hydroxy-3'-carbazol-carboxyl-amino)-4-chloro-benzene.                                                 | Brown.                                                |

|    | Diazo-component:                                                                                                                                                                                                                            | Coupling component:                                                                                                                                                                                                                                                                                                                                                                                                                                                                                                                                                                                                                                                                                                                           | Shade:                                                                                                                                             |
|----|---------------------------------------------------------------------------------------------------------------------------------------------------------------------------------------------------------------------------------------------|-----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|----------------------------------------------------------------------------------------------------------------------------------------------------|
| 5  | 4'-chloro-phenyl-4-methoxy-3-amino-benzyl-sulfone<br>Do.<br>Do.<br>Do.<br>Do.                                                                                                                                                               | (2'-hydroxy-3'-naphthoyl-amino)-benzene<br>1-(2'-hydroxy-3'-naphthoyl-amino)-2-methoxy-benzene<br>2-(2'-hydroxy-3'-naphthoyl-amino)-naphthalene<br>1-(2'-hydroxy-3'-naphthoyl-amino)-naphthalene<br>1-(2'-hydroxy-3'-naphthoyl-amino)-3-nitrobenzene<br>(2'-hydroxy-3'-naphthoyl-amino)-benzene<br>1-(2'-hydroxy-3'-naphthoyl-amino)-benzene<br>1-(2'-hydroxy-3'-naphthoyl-amino)-4-chloro-benzene<br>1-(2'-hydroxy-3'-naphthoyl-amino)-4-methyl-benzene<br>2-acetoacetylamino-6-benzoyl-amino-benzthiazol<br>1-(2'-hydroxy-3'-naphthoyl-amino)-2-methoxy-benzene<br>1-(2'-hydroxy-3'-naphthoyl-amino)-2,5-dimethoxy-4-chloro-benzene<br>1-(2'-hydroxy-3'-naphthoyl-amino)-4-ethoxy-benzene<br>2-acetoacetylamino-6-benzoyl-amino-benzthiazol | Very bright red.<br>Do.<br>Do.<br>Vivid bluish red.<br>Do.<br>Red.<br>Vivid scarlet.<br>Yellowish scarlet.<br>Do.<br>Yellow.<br>Bluish red.<br>Do. |
| 10 | 4'-methylphenyl-4-amino-benzyl-sulfone<br>Phenyl-2-amino-benzyl-sulfone<br>Do.<br>3'-chlorophenyl-2-amino-benzyl-sulfone<br>Do.<br>2'-chlorophenyl-2-amino-benzyl-sulfone<br>Do.                                                            |                                                                                                                                                                                                                                                                                                                                                                                                                                                                                                                                                                                                                                                                                                                                               | 10                                                                                                                                                 |
| 15 | 3',4'-dichloro-phenyl-2-amino-benzyl-sulfone<br>Do.                                                                                                                                                                                         |                                                                                                                                                                                                                                                                                                                                                                                                                                                                                                                                                                                                                                                                                                                                               |                                                                                                                                                    |
| 20 | 4'-chloro-phenyl-2-amino-6-chloro-benzyl-sulfone<br>Do.<br>4'-bromo-phenyl-2-amino-benzyl-sulfone<br>Do.<br>4'-chloro-2',5'-dimethyl-2-amino-benzyl-sulfone<br>Do.                                                                          |                                                                                                                                                                                                                                                                                                                                                                                                                                                                                                                                                                                                                                                                                                                                               | 20                                                                                                                                                 |
| 25 | 2'-methoxyphenyl-2-amino-benzyl-sulfone<br>Do.<br>2-amino-dibenzyl-sulfone<br>Do.<br>4'-benzene-sulfo-phenyl-2-amino-benzyl-sulfone<br>Do.<br>3'-benzene-sulfo-phenyl-2-amino-benzyl-sulfone<br>Do.<br>phenyl-4-amino-benzyl-sulfone<br>Do. |                                                                                                                                                                                                                                                                                                                                                                                                                                                                                                                                                                                                                                                                                                                                               | 25                                                                                                                                                 |

30 Since an object of the present invention is to provide dyestuffs of good fastness properties, which dyestuffs are insoluble in water and alkalies, it is to be understood that the benzene nuclei of the general formulae appearing in the appended 35 claims do not contain any substituents which are known to render organic compounds soluble in water or alkalies and to tend to depreciate the fastness of the dyestuffs to alkalies. Substituents of this kind are, for instance, the sulfonic acid, the carboxylic acid and the hydroxy group.

We claim:—

1. Azodyestuffs corresponding to the general formula:



50 wherein  $R_1$  means a radicle of the benzene series and  $R_2$  a combining component of the group consisting of arylamides of acylacetic acids and ortho-hydroxy-aryl-carboxylic acids.

## 2. Azodyestuff of the formula:



65 which dyestuff yields when prepared on the fiber  
golden orange shades of a good fastness.

### 3. Azodyestuff of the formula:



which dyestuff yields when prepared on the fiber golden orange shades of a good fastness.

4. Azodyestuff of the formula:



which dyestuff yields when prepared on the fiber 55 bright scarlet shades of a good fastness.

5. Fibers dyed with the dyestuffs claimed in claim 1.

6. Fibers dyed with the dyestuff claimed in claim 2.

7. Fibers dyed with the dyestuff claimed in

8. Fibers dyed with the dyestuff claimed in

claim 4.

WERNER ZERWECK. 65  
KARL SCHÜTZ.